

1

2,875,079

## SPINNING SOLUTION

Robert E. Clark, Madison, Tenn., assignor to E. I. du Pont de Nemours and Company, Wilmington, Del., a corporation of Delaware

No Drawing. Application March 4, 1957  
Serial No. 643,510

6 Claims. (Cl. 106—165)

This invention relates to a novel and useful composition of matter and to an improved method for the production of a textile filament. More particularly, it relates to a viscose spinning solution and to an improved method for the preparation of a rayon filament having a uniform high luster.

It is an object of this invention to provide a method for improving the uniformity of luster in the commercial production of lustrous textile rayon filaments. A further object is to provide a method for improving the level and uniformity of luster under process conditions where the yarn is normally unacceptable due to low and variable luster. Another object is to provide a viscose spinning solution which is suitable for the preparation of lustrous textile rayon filaments.

These objects are accomplished by the present invention which provides an improvement in the process for the preparation of a regenerated cellulose filament by extruding viscose into an acid coagulating and regenerating bath, which comprises incorporating into the viscose, prior to extruding, from at least about 0.02 to about 0.10% by weight, calculated as the sodium salt, of a soluble salt of a sulfated fatty acid having at least 10 carbon atoms and from about 0.05 to about 0.10% by weight, calculated as sodium sulfite, of a soluble sulfite. By the term "incorporating" is meant that the additives are present in the viscose at the time of extrusion into the acid bath. The additives, therefore, may be added directly to the viscose or the viscose ingredients at any stage of the viscose preparation or they may be formed in situ by the addition of other compounds which are converted by the alkali of the viscose into the soluble additives. The term "soluble" is used to designate that the additive is soluble to at least the required extent in the viscose solution. The term "sulfated fatty acid" is used to signify the reaction product of sulfuric acid and an ethylenically unsaturated or hydroxyl substituted fatty acid. These sulfated fatty acids all have the general formula



wherein  $n$  is a small whole integer and R is an aliphatic group of at least 9 carbon atoms. The preparation of these sulfated fatty acids is described in British Patent No. 293,480 and also in "The Industrial Chemistry of Fats and Waxes" by Hilditch, 2nd edition, pages 398 to 400 (1941). The salts of the sulfated fatty acids are formed by reacting the sulfated acid with an alkali metal hydroxide such as sodium or potassium hydroxide. The salt may also be formed in situ by the addition of the sulfated fatty acid directly to the viscose in which case the alkali of the viscose converts the acid to the sodium salt.

In the preferred embodiment of this invention a  $C_{18}$  fatty acid is employed. When oleic acid is sulfated the resulting compound has the structure



2

This compound is then incorporated into the viscose or the viscose ingredients, generally as the sodium salt, to give a viscose solution having the desired concentration of the sulfated fatty acid.

- 5 The soluble sulfite may be added to the viscose or viscose ingredients as sodium sulfite or sodium bisulfite or other soluble sulfite such as potassium sulfite or bisulfite. If the bisulfite is added it is converted to the sulfite by action of the alkali in the viscose. A preferred method 10 of addition of the sulfite, by reason of economy, is the addition of metabisulfite,  $Na_2S_2O_5$ , which in aqueous solution forms sodium bisulfite  $NaHSO_3$ ; the sodium bisulfite being converted to sodium sulfite,  $Na_2SO_3$ , by the alkali in the viscose.
- 15 The present invention also provides an improved spinning solution which comprises viscose containing at least about 0.02 to about 0.10% by weight, calculated as the sodium salt, of a soluble salt of a sulfated fatty acid having at least 10 carbon atoms and from about 20 0.05 to about 0.10% by weight, calculated as sodium sulfite, of a soluble sulfite.

The invention will now be further described in the following specific examples, which are to be regarded solely as illustrative, and not as restricting the scope of

25 the invention.

### Example 1

Alkali cellulose is prepared in the conventional manner by steeping sheets of wood pulp in caustic solution, 30 pressing to remove the excess caustic and shredding. The alkali cellulose is aged and then xanthated using 33% carbon disulfite, based on the air dried weight of the pulp. The xanthate is dissolved in dilute sodium hydroxide solution to form viscose containing 7.0% recoverable cellulose and 6.0% alkali, calculated as sodium hydroxide. During mixing 0.05% of the sodium salt 35 of sulfated oleic acid (sold under the trade name of "Prestab Oil V" and sufficient sodium metabisulfite,  $Na_2S_2O_5$ , to form 0.074% sodium sulfite, is added to the viscose.

The viscose is filtered, deaerated and ripened to a salt index of 4.5 to 4.7 and a viscosity of 45 poises at which time it is extruded through a 40 hole spinneret into a coagulating and regenerating bath maintained at 52° C. and containing 9.8% sulfuric acid, 19.8% sodium sulfate and 3.5% zinc sulfate to form a yarn of 150 denier. The yarn is passed through the bath by means of suitable roller guides, then up to and around a feed wheel and down into a centrifugal spinning bucket where it is wound into a cake at a speed of 100 yards per minute. A small stream of water at 35° C. is applied to the yarn 50 at the feed wheel to insure good cake formation.

The cakes are washed free of acid by showering with 55 soft water, desulfurized with a dilute sodium carbonate solution according to the process of U. S. Patent 1,931,266, washed with soft water for about 4 hours to remove the desulfurizing solution and bleached with a chlorine-water bleach according to the process of U. S. Patent 2,116,210. The cakes are then showered for about 60 4 hours with a conventional finish solution containing 0.1% soluble starch, 0.05% citric acid and 0.2% light mineral oil (liquid petrolatum), dispersed in the solution. The cakes are dried by heating in the conventional manner.

To judge the luster of the cakes, yarn from the inside, center and outside of the cake is wound on dull black cards about  $1\frac{1}{2} \times 6$  inches in size. The cards are then viewed obliquely in artificial light. The yarn, when 70 viewed in this manner, shows a high degree of uniformity, and substantially all of the cakes so prepared are commercially acceptable.

3  
*Example 2*

The procedure of Example 1 is again followed omitting both the sodium salt of sulfated oleic acid and the sodium metabisulfite. The yarn prepared in this manner shows a low level of luster and a low degree of uniformity. Substantially all of the cakes are commercially unacceptable.

4  
*Example 3*

The procedure of Example 1 is again followed using 0.10% of the sodium salt of sulfated oleic acid (sold under the trade name of "Prestabit Oil V"). The sodium metabisulfite is omitted in this example. Foaming occurs during the deaeration step and it is too severe to permit commercial operation of the process. In addition, a substantial number of the cakes prepared in this manner proved to be unacceptable with regard to luster uniformity and level.

5  
*Example 4*

The procedure of Example 1 is again followed using sufficient metabisulfite to form 0.15% sodium sulfite in the viscose. The sodium salt of sulfated oleic acid is, however, omitted. Difficulty is encountered in the spinning step of the process due to slow coagulation and excessive formation of sulfur sludge also occurs. A substantial number of the cakes prepared in this manner also proved to be unacceptable with regard to luster uniformity and level.

The examples thus show that yarns spun from viscose containing the sulfated fatty acid and sulfite in accordance with this invention are superior with regard to level and uniformity of luster as compared to yarns spun in the absence of these compounds or with only one of them present.

While the addition of a sulfated fatty acid and a soluble sulfite in accordance with this invention is useful in all the conventional viscose spinning processes, it is particularly useful in processes designed to produce yarns of higher strength and higher silk factor. Such processes involve the use of higher than normal concentrations of  $CS_2$ , higher salt index and/or higher than normal concentrations of metal salts, such as zinc sulfate, in the bath. Since these conditions usually result in yarns of lower and more variable luster, the yarn is not commercially acceptable. By the practice of this invention, however, the luster of these yarns are improved to the extent that the yarns are commercially acceptable and the advantages of higher strength and higher silk factor may be realized. The present invention, therefore, is partic-

ularly applicable to processes wherein viscose (salt index of at least 4.2), which has been prepared with more than 31%  $CS_2$  and which contains 6 to 8% recoverable cellulose and 4 to 8% alkali, is extruded into a coagulating and regenerating bath containing 7 to 12% sulfuric acid, 15 to 25% sodium sulfate, and 2 to 10% zinc sulfate.

The yarns prepared by this invention are useful wherever conventional textile rayon yarns are used, such as wearing apparel, draperies and the like.

Many modifications will be apparent to those skilled in the art from the reading of the above without a departure from the inventive concept.

What is claimed is:

1. In the process for the preparation of a regenerated cellulose filament by extruding viscose into an acid coagulating and regenerating bath, the improvement which comprises incorporating into the viscose, prior to extruding, from at least about 0.02 to about 0.10% by weight, calculated as the sodium salt, of a soluble salt of a sulfated fatty acid having at least 10 carbon atoms, and from about 0.05 to about 0.10% by weight, calculated as sodium sulfite, of a soluble sulfite.
2. The process of claim 1 wherein the sulfated fatty acid is a sulfated fatty acid containing 18 carbon atoms.
3. The process of claim 1 wherein the sulfated fatty acid is sulfated oleic acid.
4. A spinning solution consisting essentially of viscose containing at least about 0.02 to about 0.10% by weight, calculated as the sodium salt, of a soluble salt of a sulfated fatty acid having at least 10 carbon atoms and from about 0.05 to about 0.10% by weight, calculated as sodium sulfite, of a soluble sulfite.
5. The spinning solution of claim 4 wherein the sulfated fatty acid is a sulfated fatty acid containing 18 carbon atoms.
6. The spinning solution of claim 4 wherein the sulfated fatty acid is sulfated oleic acid.

## References Cited in the file of this patent

## UNITED STATES PATENTS

- 1,575,052 Hesse et al. ----- Mar. 2, 1926  
2,064,118 Huttinger et al. ----- Dec. 15, 1936

## FOREIGN PATENTS

- 293,480 Great Britain ----- July 6, 1928

## OTHER REFERENCES

- Hilditch: "Industrial Fats and Waxes," third edition, 1949, pages 442-443.